

## UNITED STATES PATENT OFFICE

2,572,954

## ACID DYEING PROCESS USING ALKANE-SULFONIC ACIDS

Anthony M. Schwartz, Washington, D. C., assignor to Standard Oil Company, Chicago, Ill., a corporation of Indiana

No Drawing. Application July 9, 1949,  
Serial No. 103,945

7 Claims. (Cl. 8—43)

1

This invention relates to a novel process for dyeing wool, hair, and other acid-sensitive protein fibers. In one particular aspect, this invention relates to novel metallized acid dye baths and their employment in treating wool and the like. Almost all woolen goods are dyed with colors that must be applied from an acidified bath. In some cases the acidity of the bath is quite low and acetic or formic acids are used. In other cases relatively high acidity is needed to force the dyestuff onto the fiber, and sulfuric acid is commonly used for this purpose. The quantity of sulfuric acid needed may range from 1% to 10%, based on the weight of the goods. In many instances the goods must be boiled in the dyebath for as long as 2 or 3 hours, and the acid causes appreciable degradation and weakening of the wool.

The chromiferous acid dyes, of which the Neolans (Ciba) and the Chromacyls (du Pont) are representative, are noted for requiring high acid concentrations and long boiling times. In spite of these disadvantages they are widely used because of their superior fastness properties. The Neolan dyes are soluble chromium co-ordination complexes of lake-forming azo dyes. They are prepared from suitable dyes, usually from o,o'-dihydroxy azo dyes, by heating, e. g. boiling under reflux, with a salt of tervalent chromium.

It is an object of this invention to provide novel acid dye baths for dyeing wool or other acid-sensitive protein fibers. Another object of this invention is to provide acid dye baths for wool and the like wherein part or all of the sulfuric acid which is commonly employed in such baths is replaced by an alkansulfonic acid containing 1 to 4 carbon atoms, inclusive, in the alkyl group. A further object of this invention is to provide metallized acid dye baths for wool and the like comprising essentially an alkane-sulfonic acid containing 1 to 4 carbon atoms, inclusive, in the alkyl group. Yet another object of this invention is to provide level, rapid-acting acid dye baths for wool and the like which do not induce substantial degradation in the wool, hair, or other

protein-type fiber which is being dyed. Still another object of this invention is to provide acid dye baths for wool containing sulfuric acid and C<sub>1</sub>—C<sub>4</sub> alkane-sulfonic acids, which baths retain the advantages of sulfuric acid dye baths but present important advantages over sulfuric acid dye baths. These and other objects of this invention will become apparent from the ensuing description thereof.

10 I have made the surprising discovery that alkane-sulfonic acids containing 1 to 4 carbon atoms, inclusive, in the alkyl group, or their mixtures, are even more effective than sulfuric acid in forcing acid dyes onto wool fibers and, additionally, present the important advantage over sulfuric acid in causing substantially less degradation of wool fiber.

20 In the following table are presented some examples which are illustrative of the present invention. The acid dyeings of woolen fabrics were all carried out on a standard lot of 7 oz. white flannel. Two percent dye and from 1 to 8% acid (on the weight of the goods) was used. The bath ratio was 40 to 1. The weighed swatch of wool was added to the measured amount of cold water. The acid was then added and allowed to stand 5 minutes at room temperature. The bath was then warmed to 100° F., the dye added and stirred in. The bath was then brought to the boil within a period of one-half hour, and boiling was continued for one and one-half hours. The swatch was then removed, rinsed in warm water, and air dried. The rate of dyeing, the exhaust (i. e. the amount of dyestuff left in solution at the end of the boil), and the amount of dye in the rinse water were estimated visually. Three different dyes were used, all of which contain chromium bound in the dyestuff molecule by coordinate linkages. These dyes were: Chromacyl Bordeaux R (du Pont) Chromacyl Yellow N (du Pont) and Neolan Red 3B (Ciba). Strength tests were made on a Scott inclined plane tester after the samples had been subjected to 1500 cycles on a Taber Abraser instrument. The al-

2

kali solubility test, which is one of the best indexes of the amount of damage suffered by a sample of wool, was carried out according to the standard procedure as follows: A 1 gram sample of wool is dried at 110° C. and weighed accurately. It is then placed in a tube containing 100 ml. of 0.1N NaOH solution and held at 65° C. for 1 hour. The material is then rinsed in running tap water for 6 minutes, dried at 110° C. overnight, and weighed. The percentage weight loss is equal to the alkali solubility.

In the following tables the abbreviation "ASA" refers to a mixture of C<sub>1</sub>—C<sub>4</sub> alkanesulfonic acids containing a small amount of sulfuric acid, of the order of about 1 to 2 percent. This mixture of alkanesulfonic acids was prepared by the catalytic oxidation of a mixture of the corresponding disulfides with air, employing small proportions of nitrogen oxides as the catalyst, as described and claimed in U. S. Patent 2,433,395 of W. A. Proell and B. H. Shoemaker, patented December 30, 1947.

The data in Table 1 clearly show that the loss in strength suffered by wool is considerably less with the alkanesulfonic acid than with sulfuric acid. This effect is particularly important in the case of carpet yarns, upholstery fabrics, etc., where wear-resistance is paramount. It is also very important in the case of bleached wools, shrink-resistant wools and other specially finished wools which tend to lose strength in wet processing more readily than unfinished fabrics.

It was noted that 3% alkanesulfonic acid is sufficient to insure good exhaust and dye fixation, equal to that obtained with 6–8% H<sub>2</sub>SO<sub>4</sub> (run 11). Even at 8% alkanesulfonic acid, however, the alkali solubility is within allowable limits whereas 8% H<sub>2</sub>SO<sub>4</sub> causes marked degradation.

One effect of dyeing with alkanesulfonic acids as the acid constituent of the dye bath is that a slightly different dye shade is produced upon the wool than is obtained with sulfuric acid dye baths. It was believed possible that oxidative damage to the surface of the wool might be con-

TABLE 1

*Dyeing with Neolan colors. Ames 7 oz. wool flannel, scoured and carbonized*

| Run | Per Cent | Type     | Dye                  | Strength,<br>lbs./in. <sup>1</sup> | Alkali<br>Solu-<br>bility,<br>Per Cent | Warp<br>Strength,<br>lbs./in. <sup>2</sup> |
|-----|----------|----------|----------------------|------------------------------------|----------------------------------------|--------------------------------------------|
| 1   | None     | None     | None                 | 20.4                               | 8.7                                    | 27.7                                       |
| 2   | None     | do       | Chromacyl Bordeaux R | 21.0                               | 9.3                                    | —                                          |
| 3   | 1.5      | Sulfuric | do                   | —                                  | 10.8                                   | —                                          |
| 4   | 3        | do       | do                   | —                                  | 13.2                                   | 26.3                                       |
| 5   | 6        | do       | do                   | 17.7                               | 18.3                                   | —                                          |
| 6   | 8        | do       | do                   | 16.9                               | 21.2                                   | 25.6                                       |
| 7   | 6        | do       | Neolan Red 3B        | 18.9                               | 19.4                                   | —                                          |
| 8   | 6        | do       | Chromacyl Yellow N   | 18.7                               | 17.3                                   | —                                          |
| 9   | 1        | ASA      | Chromacyl Bordeaux R | 20.8                               | 9.9                                    | —                                          |
| 10  | 1.5      | ASA      | do                   | 19.7                               | 9.8                                    | —                                          |
| 11  | 3        | ASA      | do                   | 20.3                               | 10.4                                   | 26.9                                       |
| 12  | 8        | ASA      | do                   | —                                  | 11.3                                   | —                                          |
| 13  | 8        | ASA      | do                   | —                                  | 14.5                                   | 25.6                                       |
| 14  | 1        | ASA      | Chromacyl Yellow N   | 20.3                               | 9.4                                    | —                                          |
| 15  | 1        | ASA      | Neolan Red 3B        | 21.5                               | 8.5                                    | —                                          |

<sup>1</sup> After 1500 cycles on Taber Abraser instrument.

<sup>2</sup> Measured without previous abrading treatment.

It was determined that much less alkanesulfonic acid than H<sub>2</sub>SO<sub>4</sub> is needed to give a satisfactory depth of shade and dye exhaust. About 4 to 8% H<sub>2</sub>SO<sub>4</sub> is required to accomplish the same results as 1 to 3% alkanesulfonic acid. The effect on fabric strength and alkali solubility of various dyeing treatments involving alkanesulfonic acid and H<sub>2</sub>SO<sub>4</sub> is shown in Table 1. The controls show an alkali solubility of about 9% and a breaking strength of about 20.5 pounds. Eight percent H<sub>2</sub>SO<sub>4</sub> seriously degrades the fabric, bringing the breaking strength down to about 17 pounds and the alkali solubility up to over 21% (run 6). In one experiment, 8% alkanesulfonic acid gave a much more complete exhaust, caused no appreciable loss in breaking strength and increased the alkali solubility by only about 2 points, from 9% to 11% (run 12). It had roughly the same damaging effect as 1.5% H<sub>2</sub>SO<sub>4</sub>, which is far below the amount of H<sub>2</sub>SO<sub>4</sub> needed for satisfactory dyeing.

One percent alkanesulfonic acid gives a satisfactory dyeing about equivalent to that obtained with 6% H<sub>2</sub>SO<sub>4</sub> (run 9). The results show that in every case the alkanesulfonic acid causes no substantial degradation whereas H<sub>2</sub>SO<sub>4</sub>, when employed in amounts necessary for good dyeing, doubles the alkali solubility and causes a definite decrease in the breaking strength of wool fiber.

connected with the shade differences between alkanesulfonic acids and sulfuric acid, on the theory that sulfuric acid oxidizes wool sufficiently to develop a reddish shade, whereas the non-oxidizing alkanesulfonic acids do not have this effect.

Samples of the test flannel were accordingly bleached by a standard procedure using H<sub>2</sub>O<sub>2</sub>, and were then dyed in the presence of mixed C<sub>1</sub>—C<sub>4</sub> alkanesulfonic acids. The results are shown in Table 2. The bleached samples dyed a somewhat bluer shade in alkanesulfonic acid baths than with H<sub>2</sub>SO<sub>4</sub>, but the blueing effect was much less than in the case of unbleached wool. It was slightly greater, however, than the very weak blueing effect encountered with Harriet-treated wool. It is noteworthy that the initial alkali solubility of the bleached wool is high, as expected, but very little further damage occurs in dyeing with alkanesulfonic acid baths.

The results in Table 2 also show that 3% alkanesulfonic acid and 2% H<sub>2</sub>SO<sub>4</sub> used in conjunction give practically the same shade as 8% H<sub>2</sub>SO<sub>4</sub>. In many instances it is probable that even 1% H<sub>2</sub>SO<sub>4</sub> with 2 or 3% alkanesulfonic acid would give a satisfactory shade. The degree of damage afforded by this combination is still much lower than that obtained with a percentage of straight H<sub>2</sub>SO<sub>4</sub> adequate for dyeing.

TABLE 2  
Shade change of Ames 7 oz. grey wool flannel  
dyed with Chromacyl Bordeaux R

| Pre-Treatment         | Acid (Per Cent)                              | Alkali Solubility (Per Cent)   | Shade                        |
|-----------------------|----------------------------------------------|--------------------------------|------------------------------|
| None                  | 8% H <sub>2</sub> SO <sub>4</sub>            | 21.2                           | Standard bordeaux.           |
| Bleached              | None <sup>1</sup>                            | 18.9                           |                              |
| Do                    | 1% ASA                                       | 19.2                           | Bluer, same strength.        |
| Do                    | 3% ASA                                       | 19.4                           | Bluer, slightly stronger.    |
| None                  | 1% ASA + 2% H <sub>2</sub> SO <sub>4</sub>   | 13.1                           | Sl. bluer, sl. stronger.     |
| Do                    | 3% ASA + 1% H <sub>2</sub> SO <sub>4</sub>   | 13.1                           | V. sl. bluer, sl. stronger.  |
| Do                    | 2% ASA + 2% H <sub>2</sub> SO <sub>4</sub>   | 14.8                           | Do.                          |
| Do                    | 3% ASA + 2% H <sub>2</sub> SO <sub>4</sub>   | 15.1                           | Almost same shade, strength. |
| Do                    | 1% ASA (From 50% Acid)                       | V. much bluer, sl. weaker.     | V. much bluer, sl. weaker.   |
| Do                    | 1% Ethanesulfonic acid                       | Do.                            |                              |
| Do                    | 1% ASA + 10% Na <sub>2</sub> SO <sub>4</sub> | V. much bluer and much weaker. |                              |
| Do                    | 3% ASA + 10% Na <sub>2</sub> SO <sub>4</sub> | Much bluer, same strength.     |                              |
| Harriset <sup>1</sup> | 1% ASA                                       | 15.5                           | Sl. bluer, stronger.         |

<sup>1</sup> Active chlorine treatment to produce a shrink-resistant fabric.

<sup>2</sup> This sample not dyed before measuring alkali solubility.

In Table 3 are presented data concerning the color fastness to water obtained with acid dyeing baths containing varying amounts of alkanesulfonic acids (C<sub>1</sub>—C<sub>4</sub>) and sulfuric acid. The dyed fabric (2 g.) was boiled in 40 g. of water and the relative amount of the dye leached out by the water was estimated; 1 denotes the least amount that was leached. It will be noted from Table 3 that with 3% of alkanesulfonic acid, the fastness is equal to that obtained with sulfuric acid. With sulfuric acid, in any quantity down to 1.5%, the dyeings are all of about the same water fastness. With 8% of the alkanesulfonic acids the rate of dyeing is extremely rapid, the dye bath is completely exhausted in one-half hour or less and the alkali solubility of the wool is increased by only a small amount. With 8% of the alkanesulfonic acids the fastness of the dye to water is superior to that obtained with sulfuric acid.

TABLE 3

Color fastness of 7 oz. Ames grey wool flannel  
dyed with Chromacyl Bordeaux R

| Per Cent Acid Used in Dyeing                 | Relative Amount of Color in Water |
|----------------------------------------------|-----------------------------------|
| 8% ASA                                       | 1                                 |
| 3% ASA                                       | 2                                 |
| 3% ASA + 10% Na <sub>2</sub> SO <sub>4</sub> | 2                                 |
| 1.5% ASA                                     | 4                                 |
| 1% ASA                                       | 4                                 |
| 1% ASA + 10% Na <sub>2</sub> SO <sub>4</sub> | 3                                 |
| 8% H <sub>2</sub> SO <sub>4</sub>            | 2                                 |
| 6% H <sub>2</sub> SO <sub>4</sub>            | 2                                 |
| 3% H <sub>2</sub> SO <sub>4</sub>            | 2                                 |
| 1.5% H <sub>2</sub> SO <sub>4</sub>          | 2                                 |

The light-fastness of typical dyeings made with C<sub>1</sub>—C<sub>4</sub> alkanesulfonic acids and sulfuric acid was determined, the tests being carried out according to the standard procedures of the American Association of Textile Chemists and Colorists using the Weather-O-Meter instrument. The results are shown in Table 4, wherein the dyeings are given ratings of 1, 2, 3 or 4. However, the difference between 1 and 4 is very slight. The data in Table 4 show that no significant differences in light-fastness are observable in the above-mentioned test between the sulfonic acid-dyed samples and the sulfuric acid-dyed samples.

25

TABLE 4  
Relative lightfastness of wool flannel dyed with Chromacyl Bordeaux R, after 77 hours in the Weather-O-Meter

|    | Acid Used                                         | Rating (1 = Best) |
|----|---------------------------------------------------|-------------------|
| 30 | 1% ASA + 2% H <sub>2</sub> SO <sub>4</sub>        | 1                 |
|    | 3% ASA + 2% H <sub>2</sub> SO <sub>4</sub>        | 1                 |
|    | 2% ASA + 2% H <sub>2</sub> SO <sub>4</sub>        | 2                 |
|    | 3% ASA + 1% H <sub>2</sub> SO <sub>4</sub>        | 3                 |
|    | 1% ASA (Harriset wool)                            | 3                 |
|    | 6% H <sub>2</sub> SO <sub>4</sub>                 | 3                 |
|    | 8% H <sub>2</sub> SO <sub>4</sub>                 | 3                 |
|    | 1.5% H <sub>2</sub> SO <sub>4</sub>               | 3                 |
| 35 | 4% H <sub>2</sub> SO <sub>4</sub> (Harriset wool) | 4                 |
|    | 3% H <sub>2</sub> SO <sub>4</sub>                 | 4                 |
|    | 8% ASA                                            | 4                 |
|    | 3% ASA                                            | 4                 |

The data in Table 5 indicate that acetic acid cannot be substituted for C<sub>1</sub>—C<sub>4</sub> alkanesulfonic acids in mixtures with sulfuric acid in dye baths. The data clearly indicate that acetic acid, when substituted for the alkanesulfonic acids, produces inferior results as to shade, color strength and uniformity of dyeing.

45

TABLE 5  
Appearance of 7 oz. wool flannel dyed with 2% Chromacyl Bordeaux R

|    | Acid Used                                     | Uniformity of Dyeing (Microscopic Exam.) | Dye Strength <sup>1</sup> | Shade <sup>2</sup> |
|----|-----------------------------------------------|------------------------------------------|---------------------------|--------------------|
| 50 | 8% H <sub>2</sub> SO <sub>4</sub>             | Very Good                                | 4                         | 1                  |
|    | 3% ASA + 2% H <sub>2</sub> SO <sub>4</sub>    | do                                       | 1                         | 2                  |
| 55 | 3% Acetic + 2% H <sub>2</sub> SO <sub>4</sub> | Good                                     | 2-3                       | 3-4                |
|    | 8% ASA                                        | do                                       | 2-3                       | 3-4                |
|    | 8% Acetic                                     | Fair                                     | 6                         | 5-6                |
|    | 3% ASA                                        | Poor                                     | 5                         | 5-6                |
|    | 3% Acetic                                     | Very Poor                                | 7-8                       | 7-8                |
|    | 1.5% ASA                                      | do                                       | 7-8                       | 7-8                |
|    | 0.5% Acetic                                   | do                                       | 9                         | 9                  |
| 60 | 0% Acid                                       | do                                       | 10                        | 10                 |
|    | do                                            | 11                                       | 11                        | 11                 |

<sup>1</sup> 1=strongest.

<sup>2</sup> 1=desired red shade. Other numbers refer to progressively bluer shades.

65 The dye baths and process of this present invention are applicable also to chemically modified wools, particularly wools which have been rendered shrink-resistant by treatment with active chlorine, as in the Harriset process (note for example, Ind. Eng. Chem. 40, 2280-4 (December, 1948)). The chlorine-treated wool fabric has higher initial alkali solubility than untreated wool and is more easily damaged during dyeing, but can be satisfactorily dyed with less acid.

70

In Table 6 are shown the results obtained in dyeing a Harriset shrink-resistant wool fabric as compared with an untreated fabric of identical construction. The "ASA" of Table 6 refers to a mixture of C<sub>1</sub>—C<sub>4</sub> alkanesulfonic acids. It was found that only 1% of alkanesulfonic acid was required to give good dyeing of the Harriset-treated fabric, which amount of sulfonic acid causes approximately no increase in the alkali solubility of the wool. It was found that 4% of sulfuric acid was the necessary minimum to obtain satisfactory dyeing of the Harriset-treated fabric and it will be noted that this amount of sulfuric acid doubled the alkali solubility of the wool fabric. It is most important to note that the same dye shade is produced by treatment of the Harriset-treated wool with dye baths containing either the C<sub>1</sub>—C<sub>4</sub> alkanesulfonic acids or sulfuric acid. It is observed, therefore, that the use of C<sub>1</sub>—C<sub>4</sub> alkanesulfonic acids presents marked advantages over sulfuric acid in dye baths for the treatment of wool fabrics which have been rendered shrink-resistant by an active chlorinating agent such as sodium hypochlorite.

TABLE 6  
Dyeing Harriset-treated 7 oz. grey wool flannel  
with Chromacyl Bordeaux R

| Fabric                | Acid                              | Alkali Solubility, (Per Cent) | Warp Strength, lbs./in. |
|-----------------------|-----------------------------------|-------------------------------|-------------------------|
| Untreated             | None <sup>2</sup>                 | 9.4                           | -----                   |
| Do                    | 3% ASA                            | 11.2                          | 26.4                    |
| Do                    | 4% H <sub>2</sub> SO <sub>4</sub> | 16.8                          | 24.7                    |
| Harriset <sup>1</sup> | None <sup>2</sup>                 | 15.6                          | -----                   |
| Do                    | 1% ASA                            | 15.5                          | 22.3                    |
| Do                    | 4% H <sub>2</sub> SO <sub>4</sub> | 31.4                          | 20.9                    |

<sup>1</sup> The Harriset treatment is covered in U. S. Patent 2,466,095 of Frishman and Harris, patented April 12, 1949.

<sup>2</sup> These samples were not dyed before making the measurements. In dyeing Harriset shrink-resistant wool yarn with dye baths containing mixtures of 0.25 or 1% of alkanesulfonic acids and 1% of H<sub>2</sub>SO<sub>4</sub> the shades produced were about as good as those obtained with sulfuric acid alone, the exhausts were complete, the color strength was high and microscopic examination of the wool fibers indicated good levelness in dyeing.

Although I have provided illustrative examples of specific applications of my invention, it should be understood that my invention is not limited thereto. Thus, the acid dye baths and processes of my invention may be applied not only to virgin or chemically modified wool, but to animal hair in general, since such hair is known to be very similar, chemically, to wool and to be sensitive to sulfuric acid. For the present purpose it may be remarked that by acid-sensitivity I intend to denote substantial loss of strength or substantial increase in alkali solubility following upon contact of the fiber in question with 8 weight percent of sulfuric acid at normal dyeing temperatures, usually at temperatures of about 150° F. or higher. The acid dye baths and dyeing process of the present invention may also be applied to synthetic, acid-sensitive protein fibers such as regenerated casein which has been treated with formaldehyde (Aralac, for example), soybean proteins, protein fibers derived from peanuts (Ardil, for example) and nylon-type fibers. The invention is also applicable to dyeing mixed fabrics containing wool or other acid-sensitive protein-type fiber, for example, to mixed fabrics of wool and Aralac. The dye baths and process of the present invention may also be applied to silk or to mixtures of wool and silk.

It will be appreciated that the baths and dye-

ing process of the present invention are applicable to acid dye baths, in general, for wool and the like and to metallized acid dye baths which may contain chromium, copper or other metals which form coordination complexes with soluble acid dyes.

In general, I may use the quantities of dyestuff and water based on the weight of the fabric to be treated which are used in the conventional procedures for applying acid dyes and between about 1 and about 10 weight percent of the alkanesulfonic acid, optionally together with between about 0.5 and about 5 weight percent of sulfuric acid.

Having thus described my invention what I claim is:

1. A process for dyeing wool fiber, which process comprises contacting said fiber with an acid dye bath comprising essentially a metallized azo dye and between about 1 and about 10 percent by weight, based on said fiber, of an alkanesulfonic acid having 1 to 4 carbon atoms, inclusive, in the molecule.

2. A process for dyeing wool fiber, which process comprises contacting said fiber with an acid dye bath comprising essentially a metallized azo dye and between about 1 and about 10 percent by weight, based on said fiber, of a mixture of alkanesulfonic acids having 1 to 4 carbon atoms, inclusive, in the molecule.

3. A process for dyeing wool fiber, which process comprises contacting said fiber with an acid dye bath comprising essentially a chromiferous azo dye and between about 1 and about 10 percent by weight, based on said fiber, of an alkanesulfonic acid having 1 to 4 carbon atoms, inclusive, in the molecule.

4. A process for dyeing wool fiber, which process comprises contacting said fiber with an acid dye bath comprising essentially a chromiferous azo dye and between about 1 and about 10 percent by weight, based on said fiber, of a mixture of alkanesulfonic acids having 1 to 4 carbon atoms, inclusive, in the molecule.

45 5. A dye bath comprising essentially a metallized azo dyestuff and an alkanesulfonic acid having 1 to 4 carbon atoms, inclusive, in the molecule.

50 6. A dye bath comprising essentially a chromiferous azo dyestuff and an alkanesulfonic acid having 1 to 4 carbon atoms, inclusive, in the molecule.

7. A process for dyeing a shrink-resistant wool fiber which has been prepared by treatment with active chlorine, which process comprises contacting said fibers with an acid dye bath comprising essentially a chromiferous azo dye and an alkanesulfonic acid having 1 to 4 carbon atoms, inclusive, per molecule in an amount sufficient to induce substantially dye fixation upon said fiber but not in excess of about 1 percent by weight based on said fiber, whereby dyeing of said fiber without substantial increase in the alkali solubility of said fiber results.

65 ANTHONY M. SCHWARTZ.

#### REFERENCES CITED

The following references are of record in the file of this patent:

#### UNITED STATES PATENTS

| Number       | Name       | Date          |
|--------------|------------|---------------|
| 1,864,718    | Feibelmann | June 28, 1932 |
| 2,433,395    | Proell     | Dec. 30, 1947 |
| 75 2,433,396 | Proell     | Dec. 30, 1947 |

**Certificate of Correction**

Patent No. 2,572,954

October 30, 1951

**ANTHONY M. SCHWARTZ**

It is hereby certified that error appears in the printed specification of the above numbered patent requiring correction as follows:

Column 2, line 33, for "switch" read *swatch*; columns 3 and 4, Table I, last column thereof, opposite Run 6, for "25 6" read *25.6*; column 8, line 60, for "substantialy" read *substantial*;

and that the said Letters Patent should be read as corrected above, so that the same may conform to the record of the case in the Patent Office.

Signed and sealed this 4th day of March, A. D. 1952.

[SEAL]

**THOMAS F. MURPHY,**

*Assistant Commissioner of Patents.*